

## UNITED STATES PATENT OFFICE

2,241,492

## COMPRESSION-IGNITION ENGINE FUEL

Byron M. Vanderbilt, Roselle Park, N. J., assignor  
to Standard Oil Development Company, a cor-  
poration of Delaware

No Drawing. Application April 4, 1939,  
Serial No. 265,938

6 Claims. (Cl. 44—9)

This invention relates to improved compression-ignition engine fuels and is concerned particularly with improving the combustion characteristics of hydrocarbon fuels in high speed compression-ignition engines by novel ignition quality promoters.

The new fuel compositions for improved compression-ignition engine operation herein described are obtained by the use of certain nitroalkyl nitrates, more particularly, those designated by the term nitroalkyl mononitrates. These particular compounds which are nitrates or nitric esters of monohydric nitro alcohols are now found to be very effective for improving the ignition qualities of Diesel fuels, even though corresponding nitroalcohols and nitroparaffins have been entirely or relatively ineffective.

It has already been shown that in operating high speed compression-ignition engines, commonly termed Diesel engines, the ease in starting and smoothness of running depends largely on the ignition quality of the fuel. While this characteristic of a fuel is fundamentally determined by the ignition lag measured in delay of crank angle between injection and combustion of the fuel, it is appropriately and conveniently determined by a value termed the cetane number, which is the per cent by volume of normal cetane in a mixture consisting of normal cetane and alpha-methyl naphthalene having an ignition lag equivalent to that of the fuel given the cetane number rating.

A number of attempts have been made to find a substance for accelerating ignition of Diesel fuels and these have led to proposals of addition compounds called "dopes" and "primers," generally recommended on the basis that these compounds are thermally unstable, explosive, or have low spontaneous ignition temperatures. For example, peroxides, nitrates of glycerols, nitrates of glycols, and several low molecular weight alkyl nitrates, are among the proposed compounds. Of these, the alkyl nitrates and nitrites have been found somewhat effective in increasing the cetane number of Diesel fuels, but they have to be used in relatively high concentrations for desired improvement. Furthermore, such "dopes" tend to effect a substantial reduction in the flash point of the fuel, are costly and hazardous to prepare, and generally do not have satisfactory stability.

To meet the need of a more satisfactory addition compound for improving the ignition qualities of Diesel fuels, the present invention provides a type of compound more effective than the lower

alkyl nitrates which have held precedence hitherto over others for this purpose.

For the purpose of determining ignition promoting and other desired properties of nitroalkyl nitrates, a variety of these compounds were prepared according to the general scheme involving first a condensation of a nitroparaffin with an aldehyde in the presence of a base to form a nitroalcohol, which, in turn, is esterified to the nitroalkyl nitrate. Nitroparaffins from the commercially developed vapor phase reaction of lower paraffin hydrocarbons and nitric acid may be used as an initial material for the condensation. The conversion of the nitroparaffins to nitroalcohols by reaction with formaldehyde goes readily with the formation of almost quantitative yields and the esterification of the nitroalcohols is also a smoothly and safely performed reaction resulting in close to 90% to 100% of theoretical yields. The following example illustrates the general procedure followed for preparing nitroalcohols and for converting the nitroalcohol products to their corresponding nitrates:

309 g. (3 moles) of 2-nitrobutane and 30 cc. of 0.92 N sodium hydroxide were placed in a one liter 3-neck flask equipped with stirrer, thermometer, and dropping funnel. 255 g. (3 moles) of approximately 37% of formalin solution was run in over a period of twenty minutes with good mixing. The reaction was slightly exothermic and the temperature was kept at 30° C. to 35° C. by cooling with tap water. After the addition of the formaldehyde was complete, the mixture all in one phase was heated to 40° C. and allowed to stand at this temperature for two hours. The solution was cooled to room temperature and neutralized with hydrochloric acid. It was then placed in a Claisen flask and the methanol and water removed at about 200 mm. of mercury absolute. The pressure was then further reduced to 5 mm. of mercury absolute and 2-methyl-2-nitro-1-butanol was distilled. This distillate was aerated at 75° C. to polymerize color bodies, and then redistilled to obtain the nitroalcohol as a colorless liquid boiling at 98° C. at 10 mm. mercury.

In a similar manner, a number of other nitroalcohols were prepared by reacting various primary and secondary nitroparaffins with aliphatic aldehydes.

It is important to note that a primary nitroparaffin molecule having 2 or more carbon atoms may be condensed efficiently with two molecules of formaldehyde or with one molecule of formaldehyde and one molecule of a higher aliphatic

aldehyde, such as acetaldehyde, and that a secondary nitroparaffin molecule can be condensed with only one molecule of an aliphatic aldehyde to form only a monohydric nitroalcohol. The reactions and products may be represented by the following general equations and formulae:



In each of these equations, R, R' and R'' represent alkyl radicals. Formaldehyde is the least expensive aliphatic aldehyde and the only one which may be used in preparing primary nitro-alcohols. Moreover, it is the most reactive and gives the best yields. To obtain good yields of monohydric, nitroalcohols the use of formaldehyde in about a mole to mole proportion with the nitroparaffin was found sufficient. Nitromethane reacts somewhat exceptionally as it condenses with higher aldehydes, as well as with formaldehyde, to form monohydric dihydric, and even trihydric nitroalcohols.

Nitroalkyl mononitrates were prepared from the monohydric nitroalcohols and nitroalkylene dinitrates from the dihydric nitroalcohols. The procedure which may be employed is similar to that used in esterifying aliphatic alcohols. The following example is typical of the method of preparation used and results obtained:

A solution of 35.7 g. (0.3 mole) of 2-methyl-2-nitro-1-propanol in 25 cc. of chloroform was added dropwise above the surface of a mixture of 67.5 g. of 70% nitric acid (150% excess) and 118 g. of 96% sulfuric acid. Agitation was maintained at all times, and external cooling maintained the reaction mixture at  $-10^{\circ}$  to  $-5^{\circ}$  C. Addition of the alcohol was made in about 15

minutes and the mixture was agitated an additional fifteen minutes. The reaction mixture was then poured onto crushed ice and was separated into layers. The lower layer washed with water, then with 2% sodium bicarbonate, followed by a further washing with water, was heated under a partial vacuum to distill off chloroform and any adhering water and the residue in the distillation flask was finally heated to 55° C. at 10 mm. The residue consisted of 42.4 g. of practically colorless liquid nitrate amounting to substantially a 90% theoretical yield.

Although this nitration was carried out at a maximum temperature of  $-5^{\circ}\text{ C.}$ , it was found that higher temperatures could be used for the primary nitroalcohols. Somewhat lower temperatures are required in the nitration of secondary nitroalcohols. Also, the proportions of the reactants may be varied over a wide range. One cc. samples of some of the nitrates were heated with 5 cc. samples of 95% sulfuric acid to  $45^{\circ}\text{ C.}$  and showed no decomposition. Even the nitrate of 2-methyl-2-nitro-1-propanol which appeared more unstable formed no insoluble carbonaceous material or violent gas evolution in this test which undoubtedly demonstrates that the nitrates of the nitroalcohols have a stability highly advantageous in their preparation. All of the nitro-alkyl nitrates prepared are liquids at room temperature except that of 2-methyl-2-nitro-1,3-propanediol which is a solid melting at  $39^{\circ}\text{ C.}$  All of the nitro alkyl nitrates were found to be insoluble in water but soluble in most organic solvents. They are stable at  $100^{\circ}\text{ C.}$ , none showing any discoloration on being heated at this temperature for three to five minutes. All burn spontaneously when dropped on a hot plate at a temperature of  $400^{\circ}$  to  $500^{\circ}\text{ C.}$ .

40 For the sake of clarity and simplicity, classes of nitrates of nitroalcohols which come into consideration are formulated as follows:

### 1. Nitroalkyl mononitrates:



wherein R is an alkyl radical and R' and R'' are selected from the class consisting of hydrogen and alkyl radicals, the preferred branched nitro-alkyl mononitrates being represented by this formula when R'' is an alkyl radical and when R' is hydrogen.

## 2. Nitroalkylene dinitrates:



wherein R and R' are selected from the class consisting of hydrogen and alkyl radicals, the preferred dinitrates being represented by this formula when the sum of the carbon atoms in R and R' is at least 2 so that there is a total of at least 5 carbon atoms per molecule of the compound.

All of these nitroalkyl nitrates are soluble in Diesel fuels in excess of 1% by volume with the exception of the dinitrate 2-methyl-2-nitro-1,3-propanediol. Very little of this solid appeared to dissolve in a Diesel fuel even on long shaking at room temperature. Addition of approximately an equal weight of liquid nitrates such as that of

2-methyl-2-nitro-1-propanol appeared to keep the solid nitrate in solution when 0.1% to 0.4% of each was used. A 2% solution of the nitrate of 2-methyl-2-nitro-1-propanol in Diesel fuel showed no separation on being cooled to 0° C.

For testing the effectiveness of the nitroalkyl nitrates as ignition promoters, the method described in the S. A. E. Journal of 1936, page 225, was used. This test consists in matching the performance of a test sample with blends consisting of cetane and alpha-methyl naphthalene; the per cents by volume of cetane in the blend giving the same ignition quality test performance as the fuel in question was taken as the cetane number of that fuel. The Diesel fuel employed was a petroleum gas oil fraction having a cetane number of 38. Tests were made first on the nitroalcohols themselves, and it was found that less than 1% by volume of these compounds were soluble in the fuel and that their saturated solutions showed no higher cetane rating than the unmodified hydrocarbon fuel. The following table summarizes results obtained when using amyl nitrate and various nitroalkyl mononitrates and dinitrates for comparison:

pose by splitting off nitric acid to form an olefin according to the following reaction:



The dinitrates of 4 carbon atoms per molecule are definitely inferior to the mononitrates. It is interesting to note that the dinitrate of 2-ethyl-2-nitro-1,3-propanediol is much more effective than that of 2-methyl-2-nitro-1,3-propanediol, although the latter contains more nitrate per unit weight. This is strong evidence in support of the view that the dinitrates and polynitrates in general tend to be too unstable to be very effective. The dinitrates of higher hydrogen and carbon content show possibilities in low concentrations.

Further analysis of the foregoing table brings out some very interesting facts. Although nitrogen compounds containing nitrogen only in the form of a nitro group such as nitroparaffins and nitroalcohols have been found to be entirely or relatively ineffective as ignition promoters for Diesel fuels, it is clear from the data that the nitro group in combination with a nitrate group of the same molecule makes a very effective com-

|                                  | Increase of cetane number when using— |                |            | G. to raise cetane number of 1 liter of fuel 10 points | Percent N in nitrate | G. of N to raise cetane number of 1 liter of fuel 10 points | S. G. of nitrate |
|----------------------------------|---------------------------------------|----------------|------------|--------------------------------------------------------|----------------------|-------------------------------------------------------------|------------------|
|                                  | 1% by volume                          | 0.5% by volume | 4 g./liter |                                                        |                      |                                                             |                  |
| <b>Nitrate of—</b>               |                                       |                |            |                                                        |                      |                                                             |                  |
| Sec-amyl alcohol                 | 10                                    | 6.5            | 6          | 10                                                     | 10.5                 | 1.05                                                        | 1.00             |
| 2-methyl-2-nitro-1-butanol       | 17                                    | 13             | 12         | 3.2                                                    | 15.7                 | 0.50                                                        | 1.22             |
| 2-methyl-2-nitro-1-propanol      | 20                                    | 13             | 11         | 3.5                                                    | 17.1                 | 0.60                                                        | 1.28             |
| 2-nitro-1-pentanol               | 14                                    | 9              | 9          | 6.5                                                    | 15.7                 | 1.02                                                        | 1.24             |
| 2-nitro-1-butanol                | 14                                    | 11             | 11         | 3.5                                                    | 17.1                 | 0.60                                                        | 1.24             |
| <b>Dinitrate of—</b>             |                                       |                |            |                                                        |                      |                                                             |                  |
| 2-ethyl-2-nitro-1,3-propanediol  | 9                                     | 8              | 7          | †10.0                                                  | 17.6                 | †1.76                                                       | 1.44             |
| 2-methyl-2-nitro-1,3-propanediol | (*)                                   | (*)            | 4          |                                                        | 18.7                 |                                                             |                  |
|                                  |                                       |                |            |                                                        |                      | M. P. 39° C.                                                |                  |

†Value extrapolated.

\*Value not obtained due to insufficient solubility of the promoter.

In addition to the above data, a mixture of 2 g. of dinitrate of 2-methyl-2-nitro-1,3-propanediol and 1.3 g. of the nitrate of 2-methyl-2-nitro-1-propanol per one liter of the fuel raised the cetane number of the fuel by 6 points; when using 1 g. each of the two nitrates, the cetane number was raised 5 points.

The results indicate that the nitroalkyl mononitrates are more effective and more suitable for use as ignition promoters than the alkyl nitrates and even better than the nitroalkylene dinitrates. They further show that the nitroalkylene dinitrates tend to approach the nitroalkyl mononitrates in effectiveness as they increase in carbon content or when they are used in a mixture with the mononitrate.

From among the mononitrates, the branched chain isomers of 4 and 5 carbon atoms per molecule are more effective than the straight chain compounds, especially in the higher concentrations. This is believed due to the fact that the branched chain compounds having the formula:



where R and R' represent hydrocarbon radicals, are more thermally stable than those of the straight chain type which might tend to decom-

pose. This requirement is emphasized by other data which shows that a nitro-paraffin does not improve the ignition promoting effectiveness of an alkyl nitrate, when the two types of compounds are used together with a Diesel fuel.

It is to be noted from the above data that it takes about one-half as much nitrogen in the form of the nitrate of a nitroalkyl mononitrate to be as effective as nitrogen in the alkyl nitrate although one-half of the nitrogen in the former type of compound is supposedly bound in an ineffective nitro group while all the latter is present in a nitrate group. Evidently a combination of nitro and nitrate groups in a molecule is better than either singly for ignition promoting effectiveness and various other desirable properties.

In accordance with experimental data obtained, a nitrate of an aliphatic nitroalcohol may be modified to contain other functional groups and still be properly constituted for use in promoting ignition qualities of Diesel fuels, provided the hydrogen and carbon content of the compound is adequate. For example, a nitro group, a chloro group, or a thio group, may be present as an additional substituent with or in place of a second nitrate group when the compound contains at least five carbon atoms per molecule. This is illustrated very effectively by the dinitrates of nitroalcohols. The upper limit for the number of carbon atoms per molecule in these compounds

is mainly governed by their availability or feasibility of their preparation. At present, the preferred nitroalkyl mononitrate are most conveniently and economically prepared when they contain about three to eight carbon atoms per molecule, but it is possible to prepare suitable promoters of this class having as many as 20 or more carbon atoms per molecule by using aliphatic compounds derived from petroleum. The method of producing the nitroparaffins from aliphatic compounds may be varied, as for example, nitroparaffins may be obtained by reacting halogenated aliphatic hydrocarbons with metal nitrites which tend to replace halogen substituents by nitro groups; and in some instances, the nitro group may be introduced by direct nitration.

An inspection of the formula belonging to each nitrate of nitroalcohols having satisfactory ignition promoting properties establishes that a number of these compounds are characterized by containing what may be called the active grouping, designated as follows:



but even when containing this group, the compound lacks the desired promoter properties unless it contains at least five carbon atoms per molecule, if other functional substituents are present, such as a second nitrate group. On the other hand the mononitroalkyl mononitrate, are suitable if they contain less than 5 carbon atoms per molecule; although for both technical and economic reasons, the mononitroalkyl mononitrate should contain preferably from about 3 to 8 carbon atoms per molecule.

The novel ignition promoters herein described may be used with hydrocarbon fuels in amounts varying with the amount of improvement desired in the fuel. They may be used in proportions varying from a fraction of 1% to the limit of their solubility in the fuel, but from about 0.25% to about 3% by volume are the preferred concentrations of these compounds in the fuel. A 45 gas oil fraction boiling in the range of about 400° F. to 700° F. or, in general, having a suitable boiling range for use as a fuel in Diesel-type engines may be used as the hydrocarbon fuel to be improved. A narrowly cut fraction such as one boiling from about 450° F. to 600° F. or from 500° F. to 600° F. may be used. Ordinarily, the hydrocarbon fuel may be said to have a boiling range above that of gasoline and an end point below 750° F.

This invention makes commercially feasible the preparation of Diesel fuels giving satisfactory engine performance from various crude oils, gas oils, and residual fuels having low pour points, low A. P. I. gravities, and high heat values such as those prepared from naphthenic base or mixed base stocks. The combustion characteristics of even highly paraffinic hydrocarbon fractions are also enhanced by these novel ignition promoters. Small quantities of these highly effective ignition promoters may be used for adopting various mixtures of hydrocarbons for use as Diesel fuels including recycle stocks from cracking operations, non-paraffinic extracts, oils from destructive distillations of pyrobitumens or asphaltic substances, or mixtures of these with one another or with crude petroleum fractions.

Other agents for enhancing various other

qualities of the fuels may be simultaneously added without detracting substantially from ignition qualities of the fuel, such as oiliness agents, sludge dispersers, dyes, corrosion inhibitors, anti-oxidants, viscosity improvers, pour point depressants, and gum solvents. Also, other promoters of ignition qualities may be admixed, for example, alkyl nitrates, alkyl nitrites, and other nitro-type compounds.

10 Besides the increased efficiency of automotive operation gained through the use of the herein described novel ignition promoters, many other advantages are obtained through the fact that they are economically and safely prepared and handled. Also, they have the desired physical and chemical properties which makes their use satisfactory at low temperatures as well as high temperatures, especially because they do not tend to precipitate out in cold fuel, and because they do not adversely effect the flash point of the fuel.

15 It is to be understood that this invention is not to be limited by specific embodiments which are merely given by way of illustration. The appended claims define the novel features of my invention.

20 I claim:

1. An improved Diesel fuel comprising a hydrocarbon fuel and dissolved therein a minor proportion of a nitroalkyl mononitrate in a sufficient quantity to impart improved ignition qualities to the fuel.

2. A fuel for compression-ignition engines of the Diesel type comprising a hydrocarbon fuel and admixed therewith a small amount of mono-nitroalkyl mononitrate in sufficient quantity to improve ignition qualities of the fuel.

3. An improved Diesel fuel comprising a hydrocarbon fuel and admixed therewith a minor proportion of a nitroalkyl mononitrate in sufficient quantity to improve ignition qualities of the fuel, said nitroalkyl mononitrate containing 3 to 8 carbon atoms per molecule and having the formula:



40 wherein R, R' and R'' represent hydrogen atoms or alkyl substituents, at least one alkyl substituent being present.

45 5. An improved Diesel fuel comprising a hydrocarbon fuel and admixed therewith a minor proportion of a nitroalkyl mononitrate in sufficient quantity to improve ignition qualities of the fuel, said alkyl mononitrate having the formula:



60 6. Where R and R' are alkyl radicals.

65 7. An improved Diesel fuel comprising a hydrocarbon fuel having admixed therewith a minor proportion of the nitrate of 2-nitro-1-butanol in sufficient amount to improve ignition qualities of the fuel.

80 8. An improved Diesel fuel comprising a hydrocarbon fuel having admixed therewith a minor proportion of the nitrate of 2-methyl-2-nitro-1-propanol in sufficient amount to improve ignition qualities of the fuel.

BYRON M. VANDERBILT.